



US011177069B2

(12) **United States Patent**  
**Kuniyoshi**

(10) **Patent No.:** **US 11,177,069 B2**  
(45) **Date of Patent:** **\*Nov. 16, 2021**

(54) **METHOD FOR PRODUCING R-T-B SYSTEM SINTERED MAGNET**

(71) Applicant: **HITACHI METALS, LTD.**, Tokyo (JP)

(72) Inventor: **Futoshi Kuniyoshi**, Mishima-gun (JP)

(73) Assignee: **HITACHI METALS, LTD.**, Tokyo (JP)

(\*) Notice: Subject to any disclaimer, the term of this patent is extended or adjusted under 35 U.S.C. 154(b) by 808 days.

This patent is subject to a terminal disclaimer.

(21) Appl. No.: **15/548,466**

(22) PCT Filed: **Jul. 20, 2016**

(86) PCT No.: **PCT/JP2016/071244**

§ 371 (c)(1),  
(2) Date: **Aug. 3, 2017**

(87) PCT Pub. No.: **WO2017/018291**

PCT Pub. Date: **Feb. 2, 2017**

(65) **Prior Publication Data**

US 2018/0240590 A1 Aug. 23, 2018

(30) **Foreign Application Priority Data**

Jul. 30, 2015 (JP) ..... JP2015-150585  
Feb. 16, 2016 (JP) ..... JP2016-026583

(51) **Int. Cl.**

**H01F 41/02** (2006.01)  
**B22F 3/24** (2006.01)

(Continued)

(52) **U.S. Cl.**

CPC ..... **H01F 41/0293** (2013.01); **B22F 3/1007** (2013.01); **B22F 3/24** (2013.01);

(Continued)

(58) **Field of Classification Search**

CPC .. H01F 41/0293; H01F 41/02; H01F 41/0266; H01F 1/057; H01F 1/0577;  
(Continued)

(56) **References Cited**

U.S. PATENT DOCUMENTS

8,846,136 B2 \* 9/2014 Shoji ..... H01F 1/0577  
148/302  
2010/0119703 A1 \* 5/2010 Sagawa ..... C22C 38/16  
427/127  
(Continued)

FOREIGN PATENT DOCUMENTS

JP 09-129424 A 5/1997  
JP 2012-094813 A 5/2012  
(Continued)

OTHER PUBLICATIONS

Official Communication issued in International Patent Application No. PCT/JP2016/071244, dated Oct. 4, 2016.

Primary Examiner — Alexandra M Moore

(74) Attorney, Agent, or Firm — Keating & Bennett, LLP

(57) **ABSTRACT**

A sintered R-T-B based magnet work contains R: 27.5 to 35.0 mass % (R is at least one rare-earth element which always includes Nd), B: 0.80 to 0.99 mass %, Ga: 0 to 0.8 mass %, M: 0 to 2 mass % (M is at least one of Cu, Al, Nb and Zr), and a balance T (T is at least one transition metal element which always includes Fe, with 10% or less of Fe replaceable by Co).  $[T]/55.85 > 14[B]/10.8$  is satisfied where [T] is the T content (mass %) and [B] is the B content (mass %). At least a portion of a Pr—Ga alloy is in contact with a portion of the sintered magnet work surface, and a first heat treatment is performed at a temperature between 600° C. and 950° C. A second heat treatment is performed at a temperature lower than the temperature of the first heat treatment and between 450° C. and 750° C.

**6 Claims, 2 Drawing Sheets**



|      |                                       |                                                                                                                                                                                                                                                                                                                                                                                                                                                                                                                                                                                                                                                                                                                                         |                                                                                                                                                                                                                                              |
|------|---------------------------------------|-----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|----------------------------------------------------------------------------------------------------------------------------------------------------------------------------------------------------------------------------------------------|
| (51) | <b>Int. Cl.</b>                       |                                                                                                                                                                                                                                                                                                                                                                                                                                                                                                                                                                                                                                                                                                                                         | 3/24; B22F 2999/00; B22F 2003/248; B22F 2201/20; B22F 2202/05; B22F 2301/355; C21D 6/00; C22C 38/00; C22C 38/005; C22C 38/06; C22C 38/10; C22C 38/12; C22C 38/14; C22C 38/16; C22C 28/00; C22C 2202/02; C22C 1/0433; C22C 33/0278; C22F 1/00 |
|      | <i>H01F 1/057</i>                     | (2006.01)                                                                                                                                                                                                                                                                                                                                                                                                                                                                                                                                                                                                                                                                                                                               |                                                                                                                                                                                                                                              |
|      | <i>C22C 38/00</i>                     | (2006.01)                                                                                                                                                                                                                                                                                                                                                                                                                                                                                                                                                                                                                                                                                                                               |                                                                                                                                                                                                                                              |
|      | <i>H01F 1/08</i>                      | (2006.01)                                                                                                                                                                                                                                                                                                                                                                                                                                                                                                                                                                                                                                                                                                                               |                                                                                                                                                                                                                                              |
|      | <i>C22F 1/00</i>                      | (2006.01)                                                                                                                                                                                                                                                                                                                                                                                                                                                                                                                                                                                                                                                                                                                               |                                                                                                                                                                                                                                              |
|      | <i>C21D 6/00</i>                      | (2006.01)                                                                                                                                                                                                                                                                                                                                                                                                                                                                                                                                                                                                                                                                                                                               |                                                                                                                                                                                                                                              |
|      | <i>C22C 28/00</i>                     | (2006.01)                                                                                                                                                                                                                                                                                                                                                                                                                                                                                                                                                                                                                                                                                                                               |                                                                                                                                                                                                                                              |
|      | <i>C22C 33/02</i>                     | (2006.01)                                                                                                                                                                                                                                                                                                                                                                                                                                                                                                                                                                                                                                                                                                                               |                                                                                                                                                                                                                                              |
|      | <i>C22C 1/04</i>                      | (2006.01)                                                                                                                                                                                                                                                                                                                                                                                                                                                                                                                                                                                                                                                                                                                               |                                                                                                                                                                                                                                              |
|      | <i>H01F 1/03</i>                      | (2006.01)                                                                                                                                                                                                                                                                                                                                                                                                                                                                                                                                                                                                                                                                                                                               |                                                                                                                                                                                                                                              |
|      | <i>B22F 3/10</i>                      | (2006.01)                                                                                                                                                                                                                                                                                                                                                                                                                                                                                                                                                                                                                                                                                                                               |                                                                                                                                                                                                                                              |
|      | <i>C22C 38/06</i>                     | (2006.01)                                                                                                                                                                                                                                                                                                                                                                                                                                                                                                                                                                                                                                                                                                                               |                                                                                                                                                                                                                                              |
|      | <i>C22C 38/10</i>                     | (2006.01)                                                                                                                                                                                                                                                                                                                                                                                                                                                                                                                                                                                                                                                                                                                               |                                                                                                                                                                                                                                              |
|      | <i>C22C 38/12</i>                     | (2006.01)                                                                                                                                                                                                                                                                                                                                                                                                                                                                                                                                                                                                                                                                                                                               |                                                                                                                                                                                                                                              |
|      | <i>C22C 38/14</i>                     | (2006.01)                                                                                                                                                                                                                                                                                                                                                                                                                                                                                                                                                                                                                                                                                                                               |                                                                                                                                                                                                                                              |
|      | <i>C22C 38/16</i>                     | (2006.01)                                                                                                                                                                                                                                                                                                                                                                                                                                                                                                                                                                                                                                                                                                                               |                                                                                                                                                                                                                                              |
| (52) | <b>U.S. Cl.</b>                       |                                                                                                                                                                                                                                                                                                                                                                                                                                                                                                                                                                                                                                                                                                                                         | See application file for complete search history.                                                                                                                                                                                            |
|      | CPC .....                             | <i>C21D 6/00</i> (2013.01); <i>C22C 1/0433</i> (2013.01); <i>C22C 28/00</i> (2013.01); <i>C22C 33/0278</i> (2013.01); <i>C22C 38/00</i> (2013.01); <i>C22C 38/005</i> (2013.01); <i>C22C 38/06</i> (2013.01); <i>C22C 38/10</i> (2013.01); <i>C22C 38/12</i> (2013.01); <i>C22C 38/14</i> (2013.01); <i>C22C 38/16</i> (2013.01); <i>C22F 1/00</i> (2013.01); <i>H01F 1/03</i> (2013.01); <i>H01F 1/057</i> (2013.01); <i>H01F 1/0577</i> (2013.01); <i>H01F 1/08</i> (2013.01); <i>H01F 41/02</i> (2013.01); <i>H01F 41/0266</i> (2013.01); <i>B22F 2003/248</i> (2013.01); <i>B22F 2201/20</i> (2013.01); <i>B22F 2202/05</i> (2013.01); <i>B22F 2301/355</i> (2013.01); <i>B22F 2999/00</i> (2013.01); <i>C22C 2202/02</i> (2013.01) |                                                                                                                                                                                                                                              |
| (58) | <b>Field of Classification Search</b> |                                                                                                                                                                                                                                                                                                                                                                                                                                                                                                                                                                                                                                                                                                                                         |                                                                                                                                                                                                                                              |
|      | CPC ..                                | H01F 1/08; H01F 1/03; B22F 3/1007; B22F                                                                                                                                                                                                                                                                                                                                                                                                                                                                                                                                                                                                                                                                                                 |                                                                                                                                                                                                                                              |

(56)

**References Cited**

## U.S. PATENT DOCUMENTS

|                  |         |                     |
|------------------|---------|---------------------|
| 2013/0181039 A1  | 7/2013  | Obata               |
| 2014/0132377 A1  | 5/2014  | Nakajima et al.     |
| 2014/0184370 A1  | 7/2014  | Hidaka et al.       |
| 2014/0290803 A1* | 10/2014 | Kato .....          |
|                  |         | H01F 1/0577 148/302 |
| 2015/0235747 A1  | 8/2015  | Miyamoto et al.     |
| 2016/0163434 A1  | 6/2016  | Kanada et al.       |
| 2016/0180993 A1  | 6/2016  | Kanada et al.       |
| 2016/0196904 A1* | 7/2016  | Kanada .....        |
|                  |         | C22C 38/10 420/83   |
| 2018/0025819 A1* | 1/2018  | Shigemoto .....     |
|                  |         | B22F 3/24 419/23    |
| 2018/0047504 A1* | 2/2018  | Nishiuchi .....     |
|                  |         | C22C 28/00          |

## FOREIGN PATENT DOCUMENTS

|    |                |         |
|----|----------------|---------|
| JP | 2014-086529 A  | 5/2014  |
| WO | 2012/161355 A1 | 11/2012 |
| WO | 2013/008756 A1 | 1/2013  |
| WO | 2015/020181 A1 | 2/2015  |
| WO | 2015/020182 A1 | 2/2015  |
| WO | 2015/020183 A1 | 2/2015  |

\* cited by examiner

FIG.1



FIG.2A



FIG.2B



METHOD FOR PRODUCING R-T-B SYSTEM  
SINTERED MAGNET

## TECHNICAL FIELD

The present invention relates to a method for producing a sintered R-T-B based magnet.

## BACKGROUND ART

Sintered R-T-B based magnets (where R is at least one rare-earth element which always includes Nd; where T is Fe, or Fe and Co; and B is boron) are known as permanent magnets with the highest performance, and are used in voice coil motors (VCM) of hard disk drives, various types of motors such as motors for electric vehicles (EV, HV, PHV, etc.) and motors for industrial equipment, home appliance products, and the like.

A sintered R-T-B based magnet is composed of a main phase which mainly consists of an  $R_2T_{14}B$  compound and a grain boundary phase which is at the grain boundaries of the main phase. The main phase, i.e., the  $R_2T_{14}B$  compound, is a ferromagnetic material having high saturation magnetization and an anisotropy field, and provides a basis for the properties of a sintered R-T-B based magnet.

Coercivity  $H_{cJ}$  (which hereinafter may be simply referred to as " $H_{cJ}$ ") of sintered R-T-B based magnets decreases at high temperatures, thus causing an irreversible flux loss. For this reason, sintered R-T-B based magnets for use in motors for electric vehicles, in particular, are required to have high  $H_{cJ}$ .

It is known that  $H_{cJ}$  is improved if a light rare-earth element RL (e.g., Nd or Pr) contained in the R of the  $R_2T_{14}B$  compound of a sintered R-T-B based magnet is partially replaced with a heavy rare-earth element RH (e.g., Dy or Tb).  $H_{cJ}$  is more improved as the amount of substituted RH increases.

However, replacing RL in the  $R_2T_{14}B$  compound with RH may improve the  $H_{cJ}$  of the sintered R-T-B based magnet, but decrease its remanence  $B_r$  (which hereinafter may be simply referred to as "B<sub>r</sub>"). Moreover, RHs, in particular Dy and the like, are scarce resource, and they yield only in limited regions. For this and other reasons, they have problems of instable supply, significantly fluctuating prices, and so on. Therefore, in recent years, there has been a desire for improved  $H_{cJ}$  while using as little RH as possible.

Patent Document 1 discloses a sintered R-T-B based rare-earth magnet which provides high coercivity while keeping the Dy content low. The composition of this sintered magnet is limited to a specific range characterized by relatively small B amounts as compared to any R-T-B type alloys which have been commonly used, and contains one or more metallic elements M selected from among Al, Ga and Cu. As a result, an  $R_2T_{17}$  phase is formed at the grain boundaries, and, from this  $R_2T_{17}$  phase, a transition metal-rich phase ( $R_5T_{13}M$ ) is formed at the grain boundaries with an increased volumetric proportion, whereby  $H_{cJ}$  is improved.

## CITATION LIST

## Patent Literature

[Patent Document 1] International Publication No. 2013/008756

## SUMMARY OF INVENTION

## Technical Problem

5 Although the sintered R-T-B based rare-earth magnet disclosed in Patent Document 1 provides high  $H_{cJ}$  while reducing the Dy content, it has a problem of greatly reduced  $B_r$ . Moreover, in recent years, there has been a desire for sintered R-T-B based magnets having even higher  $H_{cJ}$  in applications such as motors for electric vehicles.

10 Various embodiments of the present invention provide methods for producing sintered R-T-B based magnets which have high  $B_r$  and high  $H_{cJ}$  while keeping the RH content reduced.

15

## Solution to Problem

A method for producing a sintered R-T-B based magnet according to the present disclosure comprises:

20 a step of providing a sintered R-T-B based magnet work, containing

R: 27.5 to 35.0 mass % (where R is at least one rare-earth element which always includes Nd),

B: 0.80 to 0.99 mass %,

Ga: 0 to 0.8 mass %, and

25 M: 0 to 2 mass % (where M is at least one of Cu, Al, Nb and Zr), and including

30 a balance T (where T is Fe, or Fe and Co) and inevitable impurities, the sintered R-T-B based magnet work having a composition satisfying Inequality (1) below:

$$[T]/55.85 > 14[B]/10.8 \quad (1)$$

([T] is the T content by mass %; and [B] is the B content by mass %);

35 a step of providing a Pr—Ga alloy (Pr accounts for 65 to

97 mass % of the entire Pr—Ga alloy; 20 mass % or less of Pr is replaceable by Nd; and 30 mass % or less of Pr is replaceable by Dy and/or Tb. Ga accounts for 3 mass % to 35 mass % of the entire Pr—Ga alloy; and 50 mass % or less of Ga is replaceable by Cu. Inclusion of inevitable impurities is possible);

40 a step of, while allowing at least a portion of the Pr—Ga alloy to be in contact with at least a portion of a surface of the sintered R-T-B based magnet work, performing a first heat treatment at a temperature which is greater than 600° C. but equal to or less than 950° C. in a vacuum or an inert gas ambient; and

45 a step of performing a second heat treatment in a vacuum or an inert gas ambient for the sintered R-T-B based magnet work having been subjected to the first heat treatment, at a temperature which is lower than the temperature effected in the step of performing the first heat treatment but which is not less than 450° C. and not greater than 750° C.

In one embodiment, the Ga amount in the sintered R-T-B based magnet work is 0 to 0.5 mass %.

50 55 In one embodiment, the Nd content in the Pr—Ga alloy is equal to or less than the content of inevitable impurities.

In one embodiment, the sintered R-T-B based magnet having been subjected to the first heat treatment is cooled to 300° C. at a cooling rate of 5° C./minute or more, from the 60 temperature at which the first heat treatment was performed.

In one embodiment, the cooling rate is 15° C./minute or more.

## Advantageous Effects of Invention

65 According to embodiments of the present disclosure, a sintered R-T-B based magnet work is subjected to a heat

treatment while being in contact with a Pr—Ga alloy, whereby Pr and Ga can be diffused throughout the grain boundaries without hardly diffusing into the main phase. The presence of Pr promotes diffusion in the grain boundaries, thereby allowing Pr and Ga to diffuse deep in the magnet interior. This makes it possible to achieve high  $B_r$  and high  $H_{cJ}$  while reducing the RH content.

#### BRIEF DESCRIPTION OF DRAWINGS

FIG. 1 A flowchart showing example steps in a method for producing a sintered R-T-B based magnet according to the present disclosure.

FIG. 2A A partially enlarged cross-sectional view schematically showing a sintered R-T-B based magnet.

FIG. 2B A further enlarged cross-sectional view schematically showing the interior of a broken-lined rectangular region in FIG. 2A.

#### DESCRIPTION OF EMBODIMENTS

As shown in FIG. 1, a method for producing a sintered R-T-B based magnet according to the present disclosure includes step S10 of providing a sintered R-T-B based magnet work and step S20 of providing a Pr—Ga alloy. The order of step S10 of providing a sintered R-T-B based magnet work and step S20 of providing a Pr—Ga alloy may be arbitrary, and a sintered R-T-B based magnet work and a Pr—Ga alloy which have been produced in different places may be used.

The sintered R-T-B based magnet work contains R: 27.5 to 35.0 mass % (where R is at least one rare-earth element which always includes Nd)

B: 0.80 to 0.99 mass %

Ga: 0 to 0.8 mass %

M: 0 to 2 mass % (where M is at least one of Cu, Al, Nb and Zr), and includes

a balance T (where T is Fe, or Fe and Co), and inevitable impurities.

This sintered R-T-B based magnet work satisfies the following Inequality (1), where the T content (mass %) is denoted as [T] and the B content (mass %) is denoted as [B].

$$[T]/55.85 > 14[B]/10.8 \quad (1)$$

This inequality being satisfied means that the B content is smaller than the stoichiometric mole fraction in the  $R_2T_{14}B$  compound, that is, the B amount is small relative to the T amount that is consumed in forming the main phase ( $R_2T_{14}B$  compound).

The Pr—Ga alloy is an alloy of Pr in an amount of 65 to 97 mass and Ga in an amount of 3 mass % to 35 mass %. However, 20 mass % or less of Pr may be replaced by Nd. Moreover, 30 mass % or less of Pr may be replaced by Dy and/or Tb. Furthermore, 50 mass % or less of Ga may be replaced by Cu. The Pr—Ga alloy may contain inevitable impurities.

As shown in FIG. 1, the method for producing a sintered R-T-B based magnet according to the present disclosure further includes: step S30 of, while allowing at least a portion of the Pr—Ga alloy to be in contact with at least a portion of the surface of the sintered R-T-B based magnet work, performing a first heat treatment at a temperature which is greater than 600° C. but equal to or less than 950° C. in a vacuum or an inert gas ambient; and step S40 of performing a second heat treatment in a vacuum or an inert gas ambient for the sintered R-T-B based magnet work having been subjected to the first heat treatment, at a

temperature which is lower than the temperature effected in the step of performing the first heat treatment but which is not less than 450° C. and not greater than 750° C. Step S30 of performing the first heat treatment is performed before step S40 of performing the second heat treatment. Between step S30 of performing the first heat treatment and step S40 of performing the second heat treatment, any other step, e.g., a cooling step, a step of retrieving the sintered R-T-B based magnet work out of a mixture of the Pr—Ga alloy and the sintered R-T-B based magnet work, or the like may be performed.

##### 1. Mechanism

The sintered R-T-B based magnet has a structure such that powder particles of a raw material alloy have bound together through sintering, and is composed of a main phase which mainly consists of an  $R_2T_{14}B$  compound and a grain boundary phase which is at the grain boundaries of the main phase.

FIG. 2A is a partially enlarged cross-sectional view schematically showing a sintered R-T-B based magnet. FIG. 2B is a further enlarged cross-sectional view schematically showing the interior of a broken-lined rectangular region in FIG. 2A. In FIG. 2A, arrowheads indicating a length of 5  $\mu m$  are shown as an example of reference length to represent size. As shown in FIG. 2A and FIG. 2B, the sintered R-T-B based magnet is composed of a main phase which mainly consists of an  $R_2T_{14}B$  compound 12 and a grain boundary phase 14 which is at the grain boundaries of the main phase 12. Moreover, as shown in FIG. 2B, the grain boundary phase 14 includes a double grain boundary phase 14a in which two  $R_2T_{14}B$  compound grains adjoining each other, and grain boundary triple junctions 14b at which three  $R_2T_{14}B$  compound grains adjoin one another.

The main phase 12, i.e., the  $R_2T_{14}B$  compound, is a ferromagnetic material having high saturation magnetization and an anisotropy field. Therefore, in a sintered R-T-B based magnet, it is possible to improve  $B_r$  by increasing the abundance ratio of the  $R_2T_{14}B$  compound which is the main phase 12. In order to increase the abundance ratio of the  $R_2T_{14}B$  compound, the R amount, the T amount, and the B amount in the raw material alloy may be brought closer to the stoichiometric ratio of the  $R_2T_{14}B$  compound (i.e., the R amount: the T amount: the B amount=2:14:1). When the B amount or the R amount belonging in the  $R_2T_{14}B$  compound falls lower than the stoichiometric ratio, a magnetic substance such as an Fe phase or an  $R_2T_{17}$  phase occurs in the grain boundary phase 14, whereby  $H_{cJ}$  is drastically decreased. However, it has been believed that, when Ga is contained in the magnet composition, even if e.g. the B amount falls lower than the stoichiometric ratio, an R-T-Ga phase will occur at the grain boundaries instead of an Fe phase and an  $R_2T_{17}$  phase, thereby being able to suppress the decrease in  $H_{cJ}$ .

It has however been found through a study by the inventors that, when Ga is added in the raw material alloy or in a raw material alloy powder that is formed by pulverizing the raw material alloy, some of the Ga may become contained not only in the grain boundary phase 14 but also in the main phase 12, thereby lowering magnetization of the main phase 12 and consequently lowering  $B_r$ . Therefore, in order to obtain high  $B_r$ , the amount of Ga added needs to be reduced. On the other hand, if too small an amount of Ga is added, then the Fe phase and  $R_2T_{17}$  phase will remain in the grain boundary phase 14, thus lowering  $H_{cJ}$ . In other words, it has been found difficult to reconcile high  $B_r$  and high  $H_{cJ}$  in the case where Ga is added in the raw material alloy and/or in the raw material alloy powder.

Through further studies directed to solving the aforementioned problem, it has been found possible to restrain some of the Ga from being contained in the main phase **12** by allowing at least a portion of a Pr—Ga alloy to be in contact with at least a portion of the surface of the sintered R-T-B based magnet work of the aforementioned specific composition, and performing a specific heat treatment to introduce Ga into the sintered R-T-B based magnet work. Furthermore, in order for Ga to diffuse into the grain boundary phase **14**, it has been found important to allow Ga and Pr to diffuse from the sintered magnet work surface into the interior, by using a Ga-containing alloy whose main component is Pr.

As will be described with respect to the Examples described below, using Nd instead of Pr does not attain as high  $B_r$  and high  $H_{cJ}$  as in the case of using Pr. This is considered to be because, in the specific composition of the present invention, Pr is more likely to be diffused into the grain boundary phase **14** than is Nd. In other words, it is considered that Pr is a greater ability to permeate the grain boundary phase **14** than does Nd. Since Nd is also likely to permeate the main phase **12**, it is considered that use of an Nd—Ga alloy will allow some of the Ga to also be diffused into the main phase **12**. In this case, the amount of Ga to be diffused in the main phase **12** is smaller than in the case of adding Ga in the alloy or the alloy powder.

According to the present invention, by using a Pr—Ga alloy, Pr and Ga can be diffused throughout the grain boundaries without hardly diffusing into the main phase. Moreover, the presence of Pr promotes diffusion in the grain boundaries, thereby allowing Ga to diffuse deep in the magnet interior. This is the presumable reason for being able to achieve high  $B_r$  and high  $H_{cJ}$ .

## 2. Terminology

(a) Sintered R-T-B Based Magnet Work and a Sintered R-T-B Based Magnet

In the present invention, any sintered R-T-B based magnet prior to a first heat treatment or during a first heat treatment will be referred to as a “sintered R-T-B based magnet work”; any sintered R-T-B based magnet after a first heat treatment but prior to or during a second heat treatment will be referred to as a “sintered R-T-B based magnet work having been subjected to a/the first heat treatment”; and any sintered R-T-B based magnet after the second heat treatment will be simply referred to as a “sintered R-T-B based magnet”.

(R-T-Ga Phase)

An R-T-Ga phase is a compound containing R, T and Ga, a typical example thereof being an  $R_6T_{13}Ga$  compound. An  $R_6T_{13}Ga$  compound has a  $La_6Co_{11}Ga_3$  type crystal structure. An  $R_6T_{13}Ga$  compound may take the form of an  $R_6T_{13-\delta}Ga_{1+\delta}$  compound. In the case where Cu, Al and Si are contained in the sintered R-T-B based magnet, the R-T-Ga phase may be  $R_6T_{13-\delta}(Ga_{1-x-y-z}Cu_xAl_ySi_z)_{1+\delta}$ .

## 3. Reasons for the Limited Composition and so on (R)

The R content is 27.5 to 35.0 mass %. R is at least one rare-earth element which always includes Nd. If R is less than 27.5 mass %, a liquid phase will not sufficiently occur in the sintering process, and it will be difficult for the sinter to become adequately dense in texture. On the other hand, if R exceeds 35.0 mass %, effects of the present invention will be obtained, but the alloy powder during the production steps of the sinter will be very active, and considerable oxidation, ignition, etc. of the alloy powder may possibly occur; therefore, it is preferably 35 mass % or less. More preferably, R is 28 mass % to 33 mass %; and still more preferably, R is 29 mass % to 33 mass %. The RH content is preferably 5 mass % or less of the entire sintered R-T-B based magnet. According to the present invention, high  $B_r$ ,

and high  $H_{cJ}$  can be achieved without the use of RH; this makes it possible to reduce the amount of RH added even when a higher  $H_{cJ}$  is desired.

(B)

5 The B content is 0.80 to 0.99 mass %. By allowing the Pr—Ga alloy described below to be diffused in a sintered R-T-B based magnet work which has 0.80 to 0.99 mass % of B content while satisfying Inequality (1), an R-T-Ga phase can be generated. If the B content is less than 0.80 mass %,  $B_r$  may be decreased; if it exceeds 0.99 mass %, the amount of R-T-Ga phase generated may be so small that  $H_{cJ}$  may be decreased. Moreover, B may be partially replaced by C.

(Ga)

15 The Ga content in the sintered R-T-B based magnet work before Ga is diffused from the Pr—Ga alloy is 0 to 0.8 mass %. In the present invention, Ga is introduced by diffusing a Pr—Ga alloy in the sintered R-T-B based magnet work; therefore, it is ensured that the Ga amount in the sintered 20 R-T-B based magnet work is relatively small (or that no Ga is contained). If the Ga content exceeds 0.8 mass %, magnetization of the main phase may become lowered due to Ga being contained in the main phase as described above, so that high  $B_r$  may not be obtained. Preferably, the Ga content is 0.5 mass % or less. A higher  $B_r$  can be obtained. 25 (M)

The M content is 0 to 2 mass %. M is at least one of Cu, Al, Nb and Zr; although it may be 0 mass % and still the effects of the present invention will be obtained, a total of 2 30 mass % or less of Cu, Al, Nb and Zr may be contained. Cu and/or Al being contained can improve  $H_{cJ}$ . Cu and/or Al may be purposely added, or those which will be inevitably introduced during the production process of the raw material or alloy powder used may be utilized (a raw material 35 containing Cu and/or Al as impurities may be used). Moreover, Nb and/or Zr being contained will suppress abnormal grain growth of crystal grains during sintering. Preferably, M always contains Cu, such that Cu is contained in an amount of 0.05 to 0.30 mass %. The reason is that Cu being 40 contained in an amount of 0.05 to 0.30 mass % will allow  $H_{cJ}$  to be improved.

(Balance T)

The balance, T (where T is Fe, or Fe and Co), satisfies 45 Inequality (1). Preferably, 90% or more by mass ratio of T is Fe. Fe may be partially replaced by Co. However, if the amount of substituted Co exceeds 10% by mass ratio of the entire T,  $B_r$  will be decreased, which is not preferable. Furthermore, the sintered R-T-B based magnet work according to the present invention may contain inevitable impurities that will usually be contained in the alloy or during the production steps, e.g., didymium alloys (Nd—Pr), electrolytic iron, ferroboron, as well as small amounts of elements 50 other than the aforementioned (i.e., elements other than R, B, Ga, M and T mentioned above). For example, Ti, V, Cr, Mn, Ni, Si, La, Ce, Sm, Ca, Mg, O (oxygen), N (carbon), C (nitrogen), Mo, Hf, Ta, W, and the like may each be 55 contained.

(Inequality (1))

When Inequality (1) is satisfied, the B content is smaller 60 than in commonly-available sintered R-T-B based magnets. Commonly-available sintered R-T-B based magnets have compositions in which  $[T]/55.85$  (i.e., the atomic weight of Fe) is smaller than  $14[B]/10.8$  (i.e., the atomic weight of B), in order to ensure that an Fe phase or an  $R_2T_{17}$  phase will not 65 occur in addition to the main phase, i.e., an  $R_2T_{14}B$  phase (where [T] is the T content by mass %; and [B] is the B content by mass %). Unlike in commonly-available sintered

R-T-B based magnets, the sintered R-T-B based magnet according to the present invention is defined by Inequality (1) so that  $[T]/55.85$  (i.e., the atomic weight of Fe) is greater than  $14[B]/10.8$  (i.e., the atomic weight of B). The reason for reciting the atomic weight of Fe is that the main component of T in the sintered R-T-B based magnet according to the present invention is Fe.

(Pr—Ga Alloy)

In the Pr—Ga alloy, Pr accounts for 65 to 97 mass % of the entire Pr—Ga alloy, in which 20 mass % or less of Pr may be replaced by Nd, and 30 mass % or less of Pr may be replaced by Dy and/or Tb. Ga accounts for 3 mass % to 35 mass % of the entire Pr—Ga alloy, in which 50 mass % or less of Ga may be replaced by Cu. Inevitable impurities may be contained. In the present invention, that “20% or less of Pr may be replaced by Nd” means that, given a Pr content (mass %) in the Pr—Ga alloy being defined as 100%, 20% thereof may be replaced by Nd. For example, if Pr accounts for 65 mass % in the Pr—Ga alloy (i.e., Ga accounts for 35 mass %), then Nd may be substituted up to 13 mass %. This will result in Pr accounting for 52 mass % and Nd accounting for 13 mass %. The same also applies to Dy, Tb and Cu. Given a sintered R-T-B based magnet work which is in the composition range according to the present invention, the below-described first heat treatment may be applied to a Pr—Ga alloy in which Pr and Ga are present in the aforementioned ranges, whereby Ga can be diffused deep in the magnet interior via the grain boundaries. The present invention is characterized by the use of a Ga-containing alloy whose main component is Pr. Although Pr may be replaced by Nd, Dy and/or Tb, it should be noted that if their respective substituted amounts exceed the aforementioned ranges, there will be too little Pr to achieve high  $H_{cJ}$  and high  $H_{cJ}$ . Preferably, the Nd content in the Pr—Ga alloy is equal to or less than the content of inevitable impurities (approximately 1 mass % or less). Although 50% or less of Ga may be replaced by Cu, a decrease in  $H_{cJ}$  may result if the amount of substituted Cu exceeds 50%.

The shape and size of the Pr—Ga alloy are not particularly limited, and may be arbitrarily selected. The Pr—Ga alloy may take the shape of a film, a foil, powder, a block, particles, or the like.

4. Providing Steps

(Step of Providing a Sintered R-T-B Based Magnet Work)

A sintered R-T-B based magnet work can be provided by a generic method for producing a sintered R-T-B based magnet, such as an Nd—Fe—B type sintered magnet. As one example, a raw material alloy which is produced by a strip casting method or the like may be pulverized to not less than 1  $\mu\text{m}$  and not more than 10  $\mu\text{m}$  by using a jet mill or the like, thereafter pressed in a magnetic field, and then sintered at a temperature of not less than 900° C. and not more than 1100° C.

If the pulverized particle size (having a central value of volume as obtained by an airflow-dispersion laser diffraction method=D50) of the raw material alloy is less than 1  $\mu\text{m}$ , it becomes very difficult to produce pulverized powder, thus resulting in a greatly reduced production efficiency, which is not preferable. On the other hand, if the pulverized particle size exceeds 10  $\mu\text{m}$ , the sintered R-T-B based magnet work as finally obtained will have too large a crystal grain size to achieve high  $H_{cJ}$ , which is not preferable. So long as the aforementioned conditions are satisfied, the sintered R-T-B based magnet work may be produced from one kind of raw material alloy (a single raw-material alloy), or through a method of using two or more kinds of raw material alloys and mixing them (blend method). Moreover, the sintered

R-T-B based magnet work may contain inevitable impurities, such as O (oxygen), N (nitrogen), and C (carbon), that may exist in the raw material alloy or introduced during the production steps.

5 (Step of Providing Pr—Ga Alloy)

The Pr—Ga alloy can be provided by a method of producing a raw material alloy that is adopted in generic methods for producing a sintered R-T-B based magnet, e.g., a mold casting method, a strip casting method, a single roll 10 rapid quenching method (a melt spinning method), an atomizing method, or the like. Moreover, the Pr—Ga alloy may be what is obtained by pulverizing an alloy obtained as above with a known pulverization means such as a pin mill.

5. Heat Treatment Step

(Step of Performing First Heat Treatment)

While at least a portion of the Pr—Ga alloy is allowed to be in contact with at least a portion of the surface of the sintered R-T-B based magnet work that has been provided as above, a heat treatment is performed in a vacuum or an inert 20 gas ambient, at a temperature which is greater than 600° C. but equal to or less than 950° C. In the present invention, this heat treatment is referred to as the first heat treatment. As a result of this, a liquid phase containing Pr and Ga emerges from the Pr—Ga alloy, and this liquid phase is introduced 25 from the surface to the interior of the sintered work through diffusion, via grain boundaries in the sintered R-T-B based magnet work. This allows Ga as well as Pr to be diffused deep in the sintered R-T-B based magnet work via the grain boundaries. If the first heat treatment temperature is 600° C. 30 or less, the amount of liquid phase containing Pr and Ga may be too small to achieve high  $H_{cJ}$ ; if it exceeds 950° C.,  $H_{cJ}$  may be decreased. Preferably, the sintered R-T-B based magnet work having been subjected to the first heat treatment (greater than 600° C. but equal to or less than 940° C.) 35 is cooled to 300° C. at a cooling rate of 5° C./minute or more, from the temperature at which the first heat treatment was performed. A higher  $H_{cJ}$  can be obtained. Even more preferably, the cooling rate down to 300° C. is 15° C./minute or more.

40 The first heat treatment can be performed by placing a Pr—Ga alloy in any arbitrary shape on the sintered R-T-B based magnet work surface, and using a known heat treatment apparatus. For example, the sintered R-T-B based magnet work surface may be covered by a powder layer of the Pr—Ga alloy, and the first heat treatment may be performed. For example, after a slurry obtained by dispersing the Pr—Ga alloy in a dispersion medium is applied on the sintered R-T-B based magnet work surface, the dispersion medium may be evaporated, thus allowing the Pr—Ga 45 alloy to come in contact with the sintered R-T-B based magnet work. Examples of the dispersion medium may be alcohols (ethanol, etc.), aldehydes, and ketones.

(Step of Performing Second Heat Treatment)

A heat treatment is performed in a vacuum or an inert gas 55 ambient for the sintered R-T-B based magnet work having been subjected to the first heat treatment, at a temperature which is lower than the temperature effected in the step of performing the first heat treatment but which is not less than 450° C. and not greater than 750° C. In the present invention, this heat treatment is referred to as the second heat treatment. By performing the second heat treatment, an R-T-Ga phase is generated, whereby high  $H_{cJ}$  can be 60 achieved. If the second heat treatment is at a higher temperature than is the first heat treatment, or if the temperature of the second heat treatment is less than 450° C. or exceeds 750° C., the amount of R-T-Ga phase generated will be too small to achieve high  $H_{cJ}$ .

## Example 1

## [Providing Sintered R-T-B Based Magnet Work]

Raw materials of respective elements were weighed so as to attain the alloy compositions indicated at Nos. A-1 and A-2 in Table 1, and alloys were produced by a strip casting technique. Each resultant alloy was coarse-pulverized by a hydrogen pulverizing method, thus obtaining a coarse-pulverized powder. Next, to the resultant coarse-pulverized powder, zinc stearate was added as a lubricant in an amount of 0.04 mass % relative to 100 mass % of coarse-pulverized powder; after mixing, an airflow crusher (jet mill machine) was used to effect dry milling in a nitrogen jet, whereby a fine-pulverized powder (alloy powder) with a particle size D50 of 4  $\mu\text{m}$  was obtained. To the fine-pulverized powder, zinc stearate was added as a lubricant in an amount of 0.05 mass % relative to 100 mass % of fine-pulverized powder; after mixing, the fine-pulverized powder was pressed in a magnetic field, whereby a compact was obtained. As a pressing apparatus, a so-called orthogonal magnetic field pressing apparatus (transverse magnetic field pressing apparatus) was used, in which the direction of magnetic field application ran orthogonal to the pressurizing direction. In a vacuum, the resultant compact was sintered for 4 hours at not less than 1060° C. and not more than 1090° C. (for each sample, a temperature was selected at which a sufficiently dense texture would result through sintering), whereby a sintered R-T-B based magnet work was obtained. Each resultant sintered R-T-B based magnet work had a density of 7.5  $\text{Mg}/\text{m}^3$  or more. The components in the resultant sintered R-T-B based magnet works proved to be as shown in Table 1. The respective components in Table 1 were measured by using Inductively Coupled Plasma Optical Emission Spectroscopy (ICP-OES). Any instance of Inequality (1) according to the present invention being satisfied is indicated as “○”; any instance of failing to satisfy it is indicated as “X”. The same also applies to Tables 5, 9, 13 and 17 below. Note that each composition in Table 1 does not total to 100 mass %. This is because components (e.g., O (oxygen) and N (nitrogen)) other than the component listed in Table 1 exist. The same also applies to Tables 5, 9, 13 and 17 below.

TABLE 1

| composition of sintered R-T-B based magnet work (mass %) |      |     |     |     |      |     |     |     |     |     |     |      |                |
|----------------------------------------------------------|------|-----|-----|-----|------|-----|-----|-----|-----|-----|-----|------|----------------|
| No.                                                      | Nd   | Pr  | Dy  | Tb  | B    | Cu  | Al  | Ga  | Zr  | Nb  | Co  | Fe   | Inequality (1) |
| A-1                                                      | 30.0 | 0.0 | 0.0 | 0.0 | 0.89 | 0.1 | 0.1 | 0.0 | 0.0 | 0.0 | 1.0 | 67.1 | ○              |
| A-2                                                      | 30.0 | 1.0 | 0.0 | 0.0 | 0.89 | 0.1 | 0.1 | 0.2 | 0.0 | 0.0 | 1.0 | 67.1 | ○              |

## [Providing Pr—Ga Alloy]

Raw materials of respective elements were weighed so as to result in the alloy composition shown as No. a-1 in Table 21, and these raw materials were dissolved; thus, by a single roll rapid quenching method (melt spinning method), an alloy in ribbon or flake form was obtained. Using a mortar, the resultant alloy was pulverized in an argon ambient, and thereafter was passed through a sieve with an opening of 425  $\mu\text{m}$ , thereby providing a Pr—Ga alloy. The composition of the resultant Pr—Ga alloy is shown in Table 2.

| 5  | composition of<br>Pr—Ga alloy<br>(mass %) |    |    |
|----|-------------------------------------------|----|----|
|    | No.                                       | Pr | Ga |
| 10 | a-1                                       | 89 | 11 |

## [Heat Treatments]

15 The sintered R-T-B based magnet works of Nos. A-1 and A-2 in Table 1 were cut and ground into 7.4 mm $\times$ 7.4 mm $\times$ 4 mm cubes. Next, with respect to the sintered R-T-B based magnet work of No. A-1, on its two faces that were perpendicular to the alignment direction, 0.25 parts by mass of Pr—Ga alloy (No. a-1) was spread, relative to 100 parts by mass of sintered R-T-B based magnet work (i.e., 0.125 parts by mass per face). Thereafter, a first heat treatment was performed at a temperature shown in Table 3 in argon which was controlled to a reduced pressure of 50 Pa, followed by 20 a cooling down to room temperature, whereby a sintered R-T-B based magnet work having been subjected to the first heat treatment was obtained. Furthermore, for this sintered R-T-B based magnet work having been subjected to the first heat treatment and No. A-2 (i.e., the sintered R-T-B based magnet work which was not subjected to the first heat treatment), a second heat treatment was performed at a temperature shown in Table 3 in argon which was controlled to a reduced pressure of 50 Pa, thus producing sintered R-T-B based magnets (Nos. 1 and 2). Note that the aforementioned cooling (i.e., cooling down to room temperature after performing the first heat treatment) was conducted by introducing an argon gas in the furnace, so that an average cooling rate of 25° C./minute existed from the temperature at which the heat treatment was effected (i.e., 900° C.) to 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 89

## 11

TABLE 3

| No. | producing conditions             |                       |                    |                    |
|-----|----------------------------------|-----------------------|--------------------|--------------------|
|     | sintered R-T-B based magnet work | Pr—Ga alloy           | 1st heat treatment | 2nd heat treatment |
| 1   | A-1                              | a-1                   | 900° C.            | 500° C.            |
| 2   | A-2                              | No 1st heat treatment |                    | 500° C.            |

## [Sample Evaluations]

The resultant samples were set in a vibrating-sample magnetometer (VSM: VSM-5SC-10HF manufactured by TOEI INDUSTRY CO., LTD.) including a superconducting coil, and after applying a magnetic field up to 4 MA/m, the magnetic hysteresis curve of the sinter in the alignment direction was measured while sweeping the magnetic field to -4 MA/m. Values of  $B_r$  and  $H_{cJ}$  as obtained from the resultant hysteresis curve are shown in Table 4.

TABLE 4

| No. | $B_r$<br>(T) | $H_{cJ}$<br>(kA/m) | Notes               |
|-----|--------------|--------------------|---------------------|
| 1   | 1.40         | 1520               | present invention   |
| 2   | 1.38         | 1250               | comparative example |

As described above, although Nos. 1 and 2 are based on essentially the same composition, higher  $B_r$  and higher  $H_{cJ}$  are achieved by the embodiment of the present invention (No. 1), as indicated in Table 4. Note that examples of the present invention, including Examples described below, all attain magnetic properties as high as  $B_r \geq 1.30$  T and  $H_{cJ} \geq 1490$  kA/m.

## Example 2

A sintered R-T-B based magnet work was produced by a similar method to Example 1, except that the sintered R-T-B based magnet work was adjusted to have the composition indicated at No. B-1 in Table 5.

TABLE 5

| composition of sintered R-T-B based magnet work (mass %) |      |     |     |     |      |     |     |     |     |     |     |      |                |
|----------------------------------------------------------|------|-----|-----|-----|------|-----|-----|-----|-----|-----|-----|------|----------------|
| No.                                                      | Nd   | Pr  | Dy  | Tb  | B    | Cu  | Al  | Ga  | Zr  | Nb  | Co  | Fe   | Inequality (1) |
| B-1                                                      | 24.0 | 7.0 | 0.0 | 0.0 | 0.88 | 0.1 | 0.1 | 0.2 | 0.0 | 0.0 | 1.0 | 67.1 | ○              |

Pr—Ga alloys were produced by a similar method to Example 1, except for being adjusted so that the Pr—Ga alloys had compositions indicated at Nos. b-1 and b-2 in Table 6.

TABLE 6

| composition of Pr—Ga alloy (mass %) |    |    |    |                     |
|-------------------------------------|----|----|----|---------------------|
| No.                                 | Pr | Nd | Ga | Notes               |
| b-1                                 | 89 | 0  | 11 | present invention   |
| b-2                                 | 0  | 89 | 11 | comparative example |

## 12

After processing the sintered R-T-B based magnet work (No. B-1) in a manner similar to Example 1, the Pr—Ga alloy was spread on the sintered R-T-B based magnet work in a manner similar to No. 1 of Example 1; a first heat treatment was performed, and the sintered R-T-B based magnet work having been subjected to the first heat treatment was further subjected to a second heat treatment, thereby producing a sintered R-T-B based magnet (Nos. 3 and 4). The producing conditions (the types of sintered R-T-B based magnet work and Pr—Ga alloy and the temperatures of the first heat treatment and the second heat treatment) are shown in Table 7. Note that the cooling condition after performing the first heat treatment, down to room temperature, was similar to that of Example 1.

TABLE 7

| No. | producing conditions             |             |                    |                    |
|-----|----------------------------------|-------------|--------------------|--------------------|
|     | sintered R-T-B based magnet work | Pr—Ga alloy | 1st heat treatment | 1st heat treatment |
| 3   | B-1                              | b-1         | 850° C.            | 500° C.            |
| 4   | B-1                              | b-2         | 850° C.            | 500° C.            |

Each resultant sample was processed similarly to Example 1, and subjected to measurement under a similar method, thus determining  $B_r$  and  $H_{cJ}$ . The results are shown in Table 8.

TABLE 8

| No. | $B_r$<br>(T) | $H_{cJ}$<br>(kA/m) | Notes               |
|-----|--------------|--------------------|---------------------|
| 3   | 1.37         | 1620               | present invention   |
| 4   | 1.37         | 1320               | comparative example |

As shown in Table 8, No. 3, which is an embodiment of the present invention using a Pr—Ga alloy (No. b-1), attained higher  $H_{cJ}$  than did No. 4 using an Nd—Ga alloy (No. b-2).

## Example 3

Sintered R-T-B based magnet works were produced by a similar method to Example 1, except that the sintered R-T-B based magnet works were adjusted to have the compositions indicated at Nos. C-1 to C-4 in Table 9.

TABLE 9

| composition of sintered R-T-B based magnet work (mass %) |      |     |     |     |      |     |     |     |     |     |     |      |                |
|----------------------------------------------------------|------|-----|-----|-----|------|-----|-----|-----|-----|-----|-----|------|----------------|
| No.                                                      | Nd   | Pr  | Dy  | Tb  | B    | Cu  | Al  | Ga  | Zr  | Nb  | Co  | Fe   | Inequality (1) |
| C-1                                                      | 24.0 | 7.0 | 0.0 | 0.0 | 0.86 | 0.1 | 0.1 | 0.2 | 0.0 | 0.0 | 1.0 | 67.1 | ○              |
| C-2                                                      | 24.0 | 7.0 | 0.0 | 0.0 | 0.88 | 0.1 | 0.1 | 0.2 | 0.0 | 0.0 | 1.0 | 67.1 | ○              |
| C-3                                                      | 23.0 | 7.0 | 0.0 | 0.0 | 0.88 | 0.1 | 0.1 | 0.2 | 0.0 | 0.0 | 0.5 | 67.1 | ○              |
| C-4                                                      | 24.0 | 7.0 | 0.0 | 0.0 | 0.84 | 0.1 | 0.2 | 0.0 | 0.0 | 0.0 | 1.0 | 67.1 | ○              |

Pr—Ga alloys were produced by a similar method to Example 1, except for being adjusted so that the Pr—Ga alloys had compositions indicated at Nos. c-1 to c-20 in Table 10.

TABLE 10

| composition of Pr—Ga alloy (mass %) |    |     |    |    |    |    |
|-------------------------------------|----|-----|----|----|----|----|
| No.                                 | Nd | Pr  | Dy | Tb | Ga | Cu |
| c-1                                 | 0  | 60  | 0  | 0  | 40 | 0  |
| c-2                                 | 0  | 65  | 0  | 0  | 35 | 0  |
| c-3                                 | 0  | 80  | 0  | 0  | 20 | 0  |
| c-4                                 | 0  | 89  | 0  | 0  | 11 | 0  |
| c-5                                 | 0  | 97  | 0  | 0  | 3  | 0  |
| c-6                                 | 0  | 100 | 0  | 0  | 0  | 0  |
| c-7                                 | 9  | 80  | 0  | 0  | 11 | 0  |
| c-8                                 | 17 | 82  | 0  | 0  | 11 | 0  |
| c-9                                 | 10 | 65  | 0  | 0  | 15 | 0  |
| c-10                                | 20 | 69  | 0  | 0  | 11 | 0  |
| c-11                                | 0  | 79  | 0  | 10 | 11 | 0  |
| c-12                                | 0  | 63  | 0  | 26 | 11 | 0  |
| c-13                                | 0  | 79  | 10 | 0  | 11 | 0  |
| c-14                                | 0  | 69  | 10 | 10 | 11 | 0  |
| c-15                                | 0  | 49  | 40 | 0  | 11 | 0  |
| c-16                                | 0  | 35  | 35 | 0  | 30 | 0  |
| c-17                                | 0  | 89  | 0  | 0  | 11 | 0  |
| c-18                                | 0  | 89  | 0  | 0  | 8  | 3  |
| c-19                                | 0  | 89  | 0  | 0  | 6  | 5  |
| c-20                                | 0  | 89  | 0  | 0  | 3  | 8  |

After processing the sintered R-T-B based magnet work (Nos. C-1 to C-4) in a manner similar to Example 1, the Pr—Ga alloy was spread on the sintered R-T-B based magnet work in a manner similar to No. 1 of Example 1; a first heat treatment was performed, and the sintered R-T-B based magnet work having been subjected to the first heat treatment was further subjected to a second heat treatment, thereby producing a sintered R-T-B based magnet (Nos. 5 to 25). The producing conditions (the types of sintered R-T-B based magnet work and Pr—Ga alloy and the temperatures of the first heat treatment and the second heat treatment) are shown in Table 11. Note that the cooling condition after performing the first heat treatment, down to room temperature, was similar to that of Example 1.

TABLE 11

| producing conditions |                                  |             |                    |                    |
|----------------------|----------------------------------|-------------|--------------------|--------------------|
| No.                  | sintered R-T-B based magnet work | Pr—Ga alloy | 1st heat treatment | 2nd heat treatment |
| 5                    | C-1                              | c-1         | 800° C.            | 500° C.            |
| 6                    | C-1                              | c-2         | 800° C.            | 500° C.            |
| 7                    | C-1                              | c-3         | 800° C.            | 500° C.            |
| 8                    | C-1                              | c-4         | 800° C.            | 500° C.            |
| 9                    | C-1                              | c-5         | 800° C.            | 500° C.            |
| 10                   | C-1                              | c-6         | 800° C.            | 500° C.            |
| 11                   | C-2                              | c-7         | 850° C.            | 500° C.            |
| 12                   | C-2                              | c-8         | 850° C.            | 500° C.            |
| 13                   | C-2                              | c-9         | 850° C.            | 500° C.            |

TABLE 11-continued

| No. | producing conditions             |             |                    |                    |
|-----|----------------------------------|-------------|--------------------|--------------------|
|     | sintered R-T-B based magnet work | Pr—Ga alloy | 1st heat treatment | 2nd heat treatment |
| 14  | C-2                              | c-10        | 850° C.            | 500° C.            |
| 15  | C-3                              | c-4         | 800° C.            | 500° C.            |
| 16  | C-3                              | c-11        | 800° C.            | 500° C.            |
| 17  | C-3                              | c-12        | 800° C.            | 500° C.            |
| 18  | C-3                              | c-13        | 800° C.            | 500° C.            |
| 19  | C-3                              | c-14        | 800° C.            | 500° C.            |
| 20  | C-3                              | c-15        | 800° C.            | 500° C.            |
| 21  | C-3                              | c-16        | 800° C.            | 500° C.            |
| 22  | C-4                              | c-17        | 900° C.            | 500° C.            |
| 23  | C-4                              | c-18        | 900° C.            | 500° C.            |
| 24  | C-4                              | c-19        | 900° C.            | 500° C.            |
| 25  | C-4                              | c-20        | 900° C.            | 500° C.            |

Each resultant sample was processed similarly to Example 1, and subjected to measurement under a similar method, thus determining  $B_r$  and  $H_{cr}$ . The results are shown in Table 12.

TABLE 12

| No. | $B_r$ (T) | $H_{cr}$ (kA/m) | Notes               |
|-----|-----------|-----------------|---------------------|
| 5   | 1.36      | 1200            | comparative example |
| 6   | 1.36      | 1500            | present invention   |
| 7   | 1.36      | 1550            | present invention   |
| 8   | 1.36      | 1630            | present invention   |
| 9   | 1.36      | 1600            | present invention   |
| 10  | 1.35      | 1250            | comparative example |
| 11  | 1.37      | 1600            | present invention   |
| 12  | 1.37      | 1580            | present invention   |
| 13  | 1.37      | 1490            | present invention   |
| 14  | 1.37      | 1370            | comparative example |
| 15  | 1.37      | 1630            | present invention   |
| 16  | 1.37      | 1700            | present invention   |
| 17  | 1.37      | 1790            | present invention   |
| 18  | 1.37      | 1650            | present invention   |
| 19  | 1.37      | 1730            | present invention   |
| 20  | 1.37      | 1250            | comparative example |
| 21  | 1.37      | 1230            | comparative example |
| 22  | 1.34      | 1580            | present invention   |
| 23  | 1.34      | 1550            | present invention   |
| 24  | 1.34      | 1550            | present invention   |
| 25  | 1.34      | 1280            | comparative example |

As shown in Table 12, Nos. 6 to 9, 11 to 13, Nos. 15 to 19, and Nos. 22 to 24, which are embodiments of the present invention, attained magnetic properties as high as  $B_r \geq 1.30$  T and  $H_{cr} \geq 1490$  kA/m. On the other hand, magnetic properties as high as  $B_r \geq 1.30$  T and  $H_{cr} \geq 1490$  kA/m were not attained by: Nos. 5 and 10, in which the Ga content in the Pr—Ga alloy was outside the range of the present invention; Nos. 14, 20 and 21, in which the amounts of substituted Nd and Dy for Pr in the Pr—Ga alloy were outside the ranges of the present invention; and No. 25, in which the amount of substituted Cu for Ga in the Pr—Ga alloy was outside the range of the present invention.

## 15

## Example 4

Sintered R-T-B based magnet works were produced by a similar method to Example 1, except that the sintered R-T-B based magnet works were adjusted to have the compositions indicated at Nos. D-1 to D-16 in Table 13.

TABLE 13

| No.  | composition of sintered R-T-B based magnet work (mass %) |      |     |     |      |     |     |     |     |     |     |      |   | Inequality (1)      | Notes |
|------|----------------------------------------------------------|------|-----|-----|------|-----|-----|-----|-----|-----|-----|------|---|---------------------|-------|
|      | Nd                                                       | Pr   | Dy  | Tb  | B    | Cu  | Al  | Ga  | Zr  | Nb  | Co  | Fe   |   |                     |       |
| D-1  | 24.0                                                     | 7.0  | 0.0 | 0.0 | 0.98 | 0.1 | 0.2 | 0.3 | 0.0 | 0.0 | 1.0 | 66.4 | X | comparative example |       |
| D-2  | 24.0                                                     | 7.0  | 0.0 | 0.0 | 0.90 | 0.1 | 0.2 | 0.3 | 0.0 | 0.0 | 1.0 | 66.5 | ○ | present invention   |       |
| D-3  | 24.0                                                     | 7.0  | 0.0 | 0.0 | 0.85 | 0.1 | 0.2 | 0.3 | 0.0 | 0.0 | 1.0 | 66.6 | ○ | present invention   |       |
| D-4  | 24.0                                                     | 7.0  | 0.0 | 0.0 | 0.80 | 0.1 | 0.2 | 0.3 | 0.0 | 0.0 | 1.0 | 66.6 | ○ | present invention   |       |
| D-5  | 24.0                                                     | 7.0  | 0.0 | 0.0 | 0.78 | 0.1 | 0.2 | 0.3 | 0.0 | 0.0 | 1.0 | 66.6 | ○ | present invention   |       |
| D-6  | 27.0                                                     | 8.0  | 0.0 | 0.0 | 0.87 | 0.1 | 0.2 | 0.3 | 0.0 | 0.0 | 1.0 | 62.5 | ○ | present invention   |       |
| D-7  | 30.0                                                     | 0.0  | 0.0 | 0.0 | 0.87 | 0.1 | 0.2 | 0.0 | 0.0 | 0.0 | 1.0 | 67.8 | ○ | present invention   |       |
| D-8  | 17.0                                                     | 13.0 | 0.0 | 0.0 | 0.87 | 0.1 | 0.2 | 0.0 | 0.0 | 0.0 | 1.0 | 67.8 | ○ | present invention   |       |
| D-9  | 24.0                                                     | 9.0  | 0.5 | 0.0 | 0.88 | 0.2 | 0.2 | 0.0 | 0.0 | 0.0 | 1.0 | 64.3 | ○ | present invention   |       |
| D-10 | 24.0                                                     | 9.0  | 0.5 | 0.0 | 0.88 | 0.2 | 0.2 | 0.2 | 0.0 | 0.0 | 1.0 | 64.1 | ○ | present invention   |       |
| D-11 | 24.0                                                     | 9.0  | 0.5 | 0.0 | 0.88 | 0.2 | 0.2 | 0.3 | 0.0 | 0.0 | 1.0 | 64.0 | ○ | present invention   |       |
| D-12 | 24.0                                                     | 9.0  | 0.5 | 0.0 | 0.88 | 0.2 | 0.2 | 0.5 | 0.0 | 0.0 | 1.0 | 63.8 | ○ | present invention   |       |
| D-13 | 24.0                                                     | 9.0  | 0.5 | 0.0 | 0.88 | 0.2 | 0.2 | 0.8 | 0.0 | 0.0 | 1.0 | 63.5 | ○ | present invention   |       |
| D-14 | 24.0                                                     | 9.0  | 0.5 | 0.0 | 0.88 | 0.2 | 0.2 | 1.2 | 0.0 | 0.0 | 1.0 | 63.1 | ○ | comparative example |       |
| D-15 | 24.0                                                     | 7.0  | 0.0 | 1.0 | 0.88 | 0.2 | 0.1 | 0.3 | 0.2 | 0.0 | 1.0 | 65.4 | ○ | present invention   |       |
| D-16 | 24.0                                                     | 7.0  | 0.0 | 1.0 | 0.88 | 0.2 | 0.1 | 0.3 | 0.0 | 0.5 | 1.0 | 65.1 | ○ | present invention   |       |

A Pr—Ga alloy was produced by a similar method to Example 1, except for being adjusted so that the Pr—Ga alloy had a composition indicated at d-1 in Table 14.

50

TABLE 14

| No. | composition of Pr—Ga alloy (mass %) |    |
|-----|-------------------------------------|----|
|     | Pr                                  | Ga |
| d-1 | 89                                  | 11 |

After processing the sintered R-T-B based magnet work (Nos. D-1 to D-16) in a manner similar to Example 1, the Pr—Ga alloy was spread on the sintered R-T-B based magnet work in a manner similar to No. 1 of Example 1; a first heat treatment was performed, and the sintered R-T-B based magnet work having been subjected to the first heat treatment was further subjected to a second heat treatment, thereby producing a sintered R-T-B based magnet (Nos. 26

## 16

to 41). The producing conditions (the types of sintered R-T-B based magnet work and Pr—Ga alloy and the temperatures of the first heat treatment and the second heat treatment) are shown in Table 15. Note that the cooling condition after performing the first heat treatment, down to room temperature, was similar to that of Example 1.

TABLE 15

| No. | producing conditions             |             |                    |                    |
|-----|----------------------------------|-------------|--------------------|--------------------|
|     | sintered R-T-B based magnet work | Pr—Ga alloy | 1st heat treatment | 2nd heat treatment |
| 26  | D-1                              | d-1         | 900° C.            | 500° C.            |
| 27  | D-2                              | d-1         | 900° C.            | 500° C.            |
| 28  | D-3                              | d-1         | 900° C.            | 500° C.            |
| 29  | D-4                              | d-1         | 900° C.            | 500° C.            |
| 30  | D-5                              | d-1         | 900° C.            | 500° C.            |
| 31  | D-6                              | d-1         | 900° C.            | 500° C.            |
| 32  | D-7                              | d-1         | 900° C.            | 500° C.            |
| 33  | D-8                              | d-1         | 900° C.            | 500° C.            |
| 34  | D-9                              | d-1         | 900° C.            | 500° C.            |
| 35  | D-10                             | d-1         | 900° C.            | 500° C.            |
| 36  | D-11                             | d-1         | 900° C.            | 500° C.            |

## 17

TABLE 15-continued

|     |                                  | producing conditions |                    |                    |
|-----|----------------------------------|----------------------|--------------------|--------------------|
| No. | sintered R-T-B based magnet work | Pr—Ga alloy          | 1st heat treatment | 2nd heat treatment |
| 37  | D-12                             | d-1                  | 900° C.            | 500° C.            |
| 38  | D-13                             | d-1                  | 900° C.            | 500° C.            |
| 39  | D-14                             | d-1                  | 900° C.            | 500° C.            |
| 40  | D-15                             | d-1                  | 900° C.            | 500° C.            |
| 41  | D-16                             | d-1                  | 900° C.            | 500° C.            |

Each resultant sample was processed similarly to Example 1, and subjected to measurement under a similar method, thus determining  $B_r$  and  $H_{cJ}$ . The results are shown in Table 16.

TABLE 16

| No. | $B_r$<br>(T) | $H_{cJ}$<br>(kA/m) | Notes               |
|-----|--------------|--------------------|---------------------|
| 26  | 1.40         | 900                | comparative example |
| 27  | 1.37         | 1570               | present invention   |
| 28  | 1.36         | 1600               | present invention   |
| 29  | 1.34         | 1580               | present invention   |
| 30  | 1.33         | 1550               | present invention   |
| 31  | 1.30         | 1750               | present invention   |
| 32  | 1.39         | 1530               | present invention   |
| 33  | 1.37         | 1700               | present invention   |
| 34  | 1.34         | 1700               | present invention   |
| 35  | 1.34         | 1730               | present invention   |
| 36  | 1.34         | 1750               | present invention   |
| 37  | 1.32         | 1680               | present invention   |
| 38  | 1.31         | 1600               | present invention   |
| 39  | 1.29         | 1580               | comparative example |
| 40  | 1.36         | 1810               | present invention   |
| 41  | 1.36         | 1830               | present invention   |

As shown in Table 16, Nos. 27 to 38 and Nos. 40 and 41, which are embodiments of the present invention, attained magnetic properties as high as  $B_r \geq 1.30$  T and  $H_{cJ} \geq 1490$  kA/m. On the other hand, magnetic properties as high as  $B_r \geq 1.30$  T and  $H_{cJ} \geq 1490$  kA/m were not attained by: No. 26, in which the composition of the sintered R-T-B based magnet work did not satisfy Inequality (1) of the present invention; and No. 39, in which the Ga content in the sintered R-T-B based magnet work was outside the range of the present invention. Moreover, as is clear from Nos. 34 to 38 (in which the Ga content in the sintered R-T-B based magnet work was 0 mass % to 0.8 mass %), the Ga content in the sintered R-T-B based magnet work is preferably 0.5 mass % or less, at which higher  $H_{cJ}$  ( $H_{cJ} \geq 1680$  kA/m) is being achieved.

## Example 5

A sintered R-T-B based magnet work was produced by a similar method to Example 1, except that the sintered R-T-B based magnet work was adjusted to have the composition indicated at No. E-1 in Table 17.

TABLE 17

| composition of sintered R-T-B based magnet work (mass %) |      |     |     |     |      |     |     |     |     |     |     |      |                |
|----------------------------------------------------------|------|-----|-----|-----|------|-----|-----|-----|-----|-----|-----|------|----------------|
| No.                                                      | Nd   | Pr  | Dy  | Tb  | B    | Cu  | Al  | Ga  | Zr  | Nb  | Co  | Fe   | Inequality (1) |
| E-1                                                      | 24.0 | 7.0 | 0.0 | 0.0 | 0.88 | 0.1 | 0.1 | 0.2 | 0.0 | 0.0 | 1.0 | 67.1 | ○              |

## 18

Pr—Ga alloys were produced by a similar method to Example 1, except for being adjusted so that the Pr—Ga alloys had compositions indicated at e-1 and e-2 in Table 18.

TABLE 18

| composition of Pr—Ga alloy<br>(mass %) |    |    |    |
|----------------------------------------|----|----|----|
| No.                                    | Pr | Ga | Cu |
| e-1                                    | 89 | 8  | 3  |
| e-2                                    | 89 | 11 | 0  |

After processing the sintered R-T-B based magnet work (No. E-1) in a manner similar to Example 1, the Pr—Ga alloy was spread on the sintered R-T-B based magnet work in a manner similar to No. 1 of Example 1; a first heat treatment was performed, and the sintered R-T-B based magnet work having been subjected to the first heat treatment was further subjected to a second heat treatment, thereby producing a sintered R-T-B based magnet (Nos. 42 to 51). The producing conditions (the types of sintered R-T-B based magnet work and Pr—Ga alloy and the temperatures of the first heat treatment and the second heat treatment) are shown in Table 19. Note that the cooling condition after performing the first heat treatment, down to room temperature, was similar to that of Example 1.

TABLE 19

| producing conditions                         |     |                |                       |                       |                     |
|----------------------------------------------|-----|----------------|-----------------------|-----------------------|---------------------|
| sintered<br>R-T-B<br>based<br>magnet<br>work |     | Pr—Ga<br>alloy | 1st heat<br>treatment | 2nd heat<br>treatment | Notes               |
| No.                                          |     |                |                       |                       |                     |
| 42                                           | E-1 | e-1            | 600° C.               | 500° C.               | present invention   |
| 43                                           | E-1 | e-2            | 800° C.               | 500° C.               | present invention   |
| 44                                           | E-1 | e-2            | 900° C.               | 500° C.               | present invention   |
| 45                                           | E-1 | e-2            | 950° C.               | 500° C.               | present invention   |
| 46                                           | E-1 | e-2            | 1050° C.              | 500° C.               | comparative example |
| 47                                           | E-1 | e-2            | 800° C.               | 700° C.               | present invention   |
| 48                                           | E-1 | e-2            | 900° C.               | 720° C.               | present invention   |
| 49                                           | E-1 | e-2            | 900° C.               | 800° C.               | comparative example |
| 50                                           | E-1 | e-2            | 900° C.               | 460° C.               | present invention   |
| 51                                           | E-1 | e-2            | 600° C.               | 400° C.               | comparative example |

Each resultant sample was processed similarly to Example 1, and subjected to measurement under a similar method, thus determining  $B_r$  and  $H_{cJ}$ . The results are shown in Table 20.

TABLE 20

| No. | $B_r$<br>(T) | $H_{cJ}$<br>(kA/m) | Notes             |
|-----|--------------|--------------------|-------------------|
| 42  | 1.36         | 1590               | present invention |
| 43  | 1.36         | 1610               | present invention |

TABLE 20-continued

| No. | B <sub>r</sub><br>(T) | H <sub>cJ</sub><br>(kA/m) | Notes               |
|-----|-----------------------|---------------------------|---------------------|
| 44  | 1.36                  | 1620                      | present invention   |
| 45  | 1.36                  | 1580                      | present invention   |
| 46  | 1.34                  | 1290                      | comparative example |
| 47  | 1.36                  | 1550                      | present invention   |
| 48  | 1.36                  | 1500                      | present invention   |
| 49  | 1.37                  | 1100                      | comparative example |
| 50  | 1.36                  | 1500                      | present invention   |
| 51  | 1.35                  | 1150                      | comparative example |

As shown in Table 20, Nos. 42 to 45, Nos. 47, 48 and 50, which are embodiments of the present invention, attained magnetic properties as high as B<sub>r</sub>≥1.30 T and H<sub>cJ</sub>≥1490 kA/m. On the other hand, magnetic properties as high as B<sub>r</sub>≥1.30 T and H<sub>cJ</sub>≥1490 kA/m were not attained by: No. 46, in which the first heat treatment was outside the range of the present invention; and Nos. 49 and 51, in which the second heat treatment was outside the range of the present invention.

#### Example 6

Sintered R-T-B based magnet works were produced by a similar method to Example 1, except that the sintered R-T-B based magnet works were adjusted to have the compositions indicated at Nos. F-1 and F-2 in Table 21.

TABLE 21

| composition of sintered R-T-B based magnet work (mass %) |      |     |     |     |      |     |     |     |     |     |     |      |                |
|----------------------------------------------------------|------|-----|-----|-----|------|-----|-----|-----|-----|-----|-----|------|----------------|
| No.                                                      | Nd   | Pr  | Dy  | Tb  | B    | Cu  | Al  | Ga  | Zr  | Nb  | Co  | Fe   | Inequality (1) |
| F-1                                                      | 19.0 | 7.0 | 0.0 | 4.0 | 0.88 | 0.1 | 0.2 | 0.5 | 0.1 | 0.0 | 1.0 | 68.2 | ○              |
| F-2                                                      | 19.0 | 7.0 | 4.0 | 0.0 | 0.88 | 0.1 | 0.2 | 0.5 | 0.1 | 0.0 | 1.0 | 68.2 | ○              |

A Pr—Ga alloy was produced by a similar method to Example 1, except for being adjusted so that the Pr—Ga alloy had a composition indicated at f-1 in Table 22.

TABLE 22

| composition of Pr—Ga alloy<br>(mass %) |    |    |    |
|----------------------------------------|----|----|----|
| No.                                    | Pr | Ga | Cu |
| f-1                                    | 89 | 11 | 0  |

After processing the sintered R-T-B based magnet work (Nos. F-1 and F-2) in a manner similar to Example 1, the Pr—Ga alloy was spread on the sintered R-T-B based magnet work in a manner similar to No. 1 of Example 1; a first heat treatment was performed, and the sintered R-T-B based magnet work having been subjected to the first heat treatment was further subjected to a second heat treatment, thereby producing a sintered R-T-B based magnet (Nos. 52 and 53). The producing conditions (the types of sintered R-T-B based magnet work and Pr—Ga alloy and the temperatures of the first heat treatment and the second heat treatment) are shown in Table 23. Note that the cooling down to room temperature after performing the first heat treatment was conducted by introducing an argon gas in the furnace, so that an average cooling rate of 10° C./minute existed from the temperature at which the heat treatment was

effected (i.e., 900° C.) to 300° C. At the average cooling rate (10° C./minute), variation in the cooling rate (i.e., a difference between the highest value and the lowest value of the cooling rate) was within 3° C./minute.

TABLE 23

| No. | producing conditions    |             |                    |                    |                   |
|-----|-------------------------|-------------|--------------------|--------------------|-------------------|
|     | sintered                |             | 1st heat treatment | 2nd heat treatment | Notes             |
|     | R-T-B based magnet work | Pr—Ga alloy |                    |                    |                   |
| 52  | F-1                     | f-1         | 900° C.            | 500° C.            | present invention |
| 53  | F-2                     | f-1         | 900° C.            | 500° C.            | present invention |

Each resultant sample was processed similarly to Example 1, and subjected to measurement under a similar method, thus determining B<sub>r</sub> and H<sub>cJ</sub>. The results are shown in Table 24.

TABLE 24

| No. | B <sub>r</sub><br>(T) | H <sub>cJ</sub><br>(kA/m) | Notes             |
|-----|-----------------------|---------------------------|-------------------|
| 52  | 1.30                  | 2480                      | present invention |
| 53  | 1.30                  | 2210                      | present invention |

As shown in Table 24, also in the case where the sintered R-T-B based magnet work contained Tb and Dy relatively profusely (4%), Nos. 52 and 53, which are embodiments of the present invention, attained high magnetic properties.

#### INDUSTRIAL APPLICABILITY

According to the present invention, a sintered R-T-B based magnet with high remanence and high coercivity can be produced. A sintered magnet according to the present invention is suitable for various motors such as motors to be mounted in hybrid vehicles, home appliance products, etc., that are exposed to high temperatures.

#### REFERENCE SIGNS LIST

- 12 main phase consisting of R<sub>2</sub>T<sub>14</sub>B compound  
14 grain boundary phase  
14a double grain boundary phase  
14b grain boundary triple junction

The invention claimed is:

1. A method for producing a sintered R-T-B based magnet, comprising:  
a step of providing a sintered R-T-B based magnet work, containing

**21**

R: 27.5 to 35.0 mass % (where R is at least one rare-earth element which always includes Nd),  
 B: 0.80 to 0.99 mass %,  
 Ga: 0 to 0.8 mass %, and  
 M: 0 to 2 mass % (where M is at least one of Cu, Al, Nb and Zr), and including  
 a balance T (where T is Fe, or Fe and Co) and inevitable impurities, the sintered R-T-B based magnet work having a composition satisfying Inequality (1) below:

$$[T]/55.85 > 14[B]/10.8 \quad (1)$$

([T] is the T content by mass %; and [B] is the B content by mass %), the sintered R-T-B based magnet work including a main phase which consists of an  $R_2T_{14}B$  compound, and including a grain boundary phase which is at grain boundaries of the main phase, wherein the sintered R-T-B based magnet work is formed by sintering particles each having a size of not less than 1  $\mu\text{m}$  and not more than 10  $\mu\text{m}$ ;  
 a step of providing a Pr—Ga alloy (Pr accounts for 65 to 97 mass % of the entire Pr—Ga alloy; 20 mass % or less of Pr is replaceable by Nd; and 30 mass % or less of Pr is replaceable by Dy and/or Tb; Ga accounts for 3 mass % to 35 mass % of the entire Pr—Ga alloy; and 50% or less of Ga is replaceable by Cu; inclusion of inevitable impurities is possible);  
 a step of, while allowing at least a portion of the Pr—Ga alloy to be in contact with at least a portion of a surface of the sintered R-T-B based magnet work, performing a first heat treatment at a temperature which is greater

10

15

20

25

**22**

than 600° C. but equal to or less than 950° C. in a vacuum or an inert gas ambient; and  
 a step of performing a second heat treatment in a vacuum or an inert gas ambient for the sintered R-T-B based magnet work having been subjected to the first heat treatment, at a temperature which is lower than the temperature effected in the step of performing the first heat treatment but which is not less than 450° C. and not greater than 750° C., wherein  
 the sintered R-T-B based magnet has a remanence  $B_r \geq 1.30 \text{ T}$  and a coercivity  $H_c \geq 1490 \text{ kA/m}$ .  
 2. The method for producing a sintered R-T-B based magnet of claim 1, wherein the Ga amount in the sintered R-T-B based magnet work is 0 to 0.5 mass %.  
 3. The method for producing a sintered R-T-B based magnet of claim 1, wherein the Nd content in the Pr—Ga alloy is equal to or less than the content of inevitable impurities.  
 4. The method for producing a sintered R-T-B based magnet of claim 1, wherein the sintered R-T-B based magnet having been subjected to the first heat treatment is cooled to 300° C. at a cooling rate of 5° C./minute or more, from the temperature at which the first heat treatment was performed.  
 5. The method for producing a sintered R-T-B based magnet of claim 4, wherein the cooling rate is 15° C./minute or more.  
 6. The method for producing a sintered R-T-B based magnet of claim 4, wherein an R-T-Ga phase is formed at the grain boundaries.

\* \* \* \* \*